

## UNITED STATES PATENT OFFICE

2,550,474

## STRESS-AGING PROCESS

Richards H. Harrington, Schenectady, N. Y., assignor to General Electric Company, a corporation of New York

No Drawing. Application September 30, 1948,  
Serial No. 52,145

15 Claims. (Cl. 148—11.5)

1

This application is a continuation-in-part of my copending application Serial No. 663,754, filed April 20, 1946, now abandoned, and assigned to the same assignee as the present invention.

The present invention is a heat treatment combined with an applied stress, for alloys and particularly alloys which are constituted either wholly or principally of one or more solid solution phases. It is one of the objects of the present invention to provide a method for improving the properties of such alloys and particularly the elastic properties and electrical conductivity. Other objects will appear hereinafter.

The novel treatment of the present invention broadly comprises heating alloys, constituted wholly or in major part of a solid solution phase (or phases) for correct times at effective elevated temperatures while the material is subjected to effective stress from an externally applied load. The resulting effects on physical properties, compared with all past experience for any of the previously known treatments, are startling, to say the least. By means of this new treatment it is possible in certain alloys (although all such alloys will be advantageously affected to some degree), to double and almost triple the elastic properties together with an increased tensile strength combined with a previously unknown simultaneous increase in elongation and increase in electrical conductivity. Considering tensile properties alone, it has heretofore been considered impossible to effect such increases in strength properties of solid solution alloys without drastic cold reduction whereas the process of the present invention does not involve any measurable plastic deformation. Also it has been previously considered impossible to obtain such increased tensile properties without coincident decrease in elongation by any known treatment, whether by cold working or by heat treatment.

Prior to the present invention, hereinafter designated a "stress-aging" process, all teaching and

experience have indicated that single phase solid solution alloys could not be given any heat treatment other than a strain relief of the cold worked materials, or an anneal, and that the only way to strengthen solid solution alloys was by cold work. The prior art teaching and experience also has indicated that such cold worked materials could not be further strengthened without further cold reduction and that all additional cold reduction was progressively less effective. In my improved process which comprises a heat treatment under applied external stress, it will be shown that such prior art teachings are erroneous and that heat treating or aging under applied external stress effects a great improvement in alloy properties.

The present process comprises heating alloys, consisting wholly or in major part of one or more solid solution phases, at temperatures below the recrystallization temperature but high enough to provide maximum diffusion while still providing a condition of elasticity in the crystal lattice, while the alloy is submitted to externally applied tension (or compression) loads of about maximum elastic value. Above the recrystallization temperature, such alloys are practically completely lacking in elasticity, are readily plastically deformed (or hot worked) and have rapid rates of creep even for the slightest loads. The loads chosen for "stress-aging" effects of maximum degree are the stresses in the range of the proportional limit, and may be as high as the 0.2% offset yield strength, determined for the alloy in its condition immediately previous to stress aging, so long as said loads do not cause measurable (destructive) creep during the stress-aging period. Of course, any processes depending upon diffusion involve time, and, as will be shown hereinafter, time at stress-aging temperature is a factor and will vary with different alloy compositions. Since stress is always measured in terms of the load per unit area, the new process is correctly named "stress-aging." However,

due to common improper confusion of the two terms "stress" and "strain," such a less useful name as "load-aging" might avoid confusion of "stress-aging" with "stress-relief," etc.

The similarity of nomenclature between "stress-relief" and "stress-aging" may be confusing solely on the basis of the language employed. However, in view of the established and present definitions, they are readily seen to be distinctively different processes for distinctively different purposes and with distinctively different property effects.

Cold worked or cast alloys are usually characterized by internal elastic strains that may cause warping after machining, etc. Strain relief (or stress relief) consists of heating the alloy to relatively low temperatures to relieve the crystal lattice of elastic distortion. In the case of cold-worked alloys, the object is to relieve this elastic lattice distortion with as little softening effect as possible, retaining as much as possible the high strength properties of the plain cold-worked condition. The tendency of strain relief treatment is to lower the strength properties and to increase the elongation. Annealing, on the other hand, consists of heating to a temperature above the recrystallization range, chiefly in order to remove all property and structure effects of previous cold work. Annealing results in minimum strength properties and maximum elongation.

The present invention, in general, may be applied to all alloys which comprise in whole or major part one or more solid solution phases. Qualitatively, rates of diffusion in metals and alloys at room temperature are proportional to the specific melting points or melting ranges, and thermal agitation of atoms within the crystal structure is proportional to temperature. Metals and alloys with higher melting points and ranges have higher recrystallization temperatures and are more stable at room temperature. Thus, cold worked alloys of aluminum, copper, nickel, iron, etc. maintain their cold worked structures at room temperature and up to higher temperatures until they definitely soften and recrystallize, whereas alloys of lead and most alloys of zinc recrystallize at or below room temperature. The practical stability, theoretically the metastability, of the stress-aged condition should parallel that of the cold worked condition. Thus, alloys which recrystallize at or below ambient temperatures cannot be stress-aged to any practical degree, that is, for subsequent applications at or above ambient temperatures.

In carrying out the present invention, alloys constituted wholly or principally of one or more solid solution phases are heated generally at temperatures well above 100° C., while external stress is applied to the alloy. The most effective stress-aging temperatures are within the range extending from somewhat below and up to the temperatures employed for softening in standard annealing, or, in other words, extends from about 100° C. below and up to the recrystallization temperature. The temperatures employed and the results obtained distinguish the present process from the phenomenon known as "strain-aging." This is a phenomenon not yet truly understood. The effects of this phenomenon have been measured and are clearly described in Metals, Carpenter and Robertson, vol. I, 1939, Oxford University Press, N. Y. C., page 174, as follows: "In general, the limit of proportionality, yield-point, and ultimate tensile strength should decrease as the temperature of testing is raised.

So far as the first two are concerned this statement is approximately true, but it is far from true when applied to the ultimate tensile strength, when the metal under consideration undergoes substantial strain-aging." Thus strain-aging is some kind of strengthening effect taking place at stresses (applied loads) high in the permanent deformation range, above the yield-point, during a tensile test at an elevated temperature within a rather critical range of temperature, which, in turn, is not close to or at all associated with the recrystallization range. Furthermore, the increased tensile strength is accompanied by a sharp decrease in elongation. Strain-aging is pronounced in iron and steels with a maximum strengthening effect at about 250° C. and is not related to the recrystallization range (450-600° C.). In most non-ferrous alloys strain-aging does not exist. A very much smaller bulge in the tensile-strength vs. testing-temperature curve for some non-ferrous alloys cannot be definitely associated with strain-aging in steel.

Applicant's process of stress-aging is carried on under constant external loads, equivalent to the proportional limit—0.2% offset yield strength range of the alloy's previous room temperature stress-strain curve, said loads being applied for extended periods of time at temperatures just below the alloy's recrystallization temperature, said stress-aging process being markedly effective on both ferrous and non-ferrous alloys, alike, in markedly increasing the subsequent room-temperature, proportional limit and yield strength of the stress-aged alloy. Thus the phenomena and results of applicant's stress-aging are obviously entirely different from those of "strain-aging."

The beneficial effect of the stress-aging process increases with increase in the applied stress, increase in aging temperature (until a temperature is reached beyond which the tendency to anneal overcomes the stress-aging reaction), and increase in the time at temperature of aging. A twenty hour aging period usually provides satisfactory results although alloys with very slow diffusion rates respond to longer aging periods. In general, an aging period of four hours achieves about 90 to 95% of the complete effect of stress-aging and in many cases an aging period of one-half hour, or even 15 minutes, will accomplish useful results.

The most effective stresses which may be employed with any alloy having a solid solution dominated structure are those which range from the proportional limit to the 0.2% off-set yield strength determined for the material in the condition preceding stress-aging. In certain cases wherein the coincident creep or flow is not appreciable still higher stresses will be found to be beneficial. Stresses lower than the proportional limit of the initial condition of the alloy are much less effective and in many cases would not justify a special treatment. Otherwise defined, for any given temperature within the prescribed range hereinbefore given, the stress should equal or exceed the proportional limit of the alloy (before stress-aging) but should not be great enough to effect a practically measurable permanent deformation at the stress-aging temperature, i. e. should not effect a permanent deformation greater than about 1 mil per inch. Alloys with higher melting ranges require greater applied stresses for maximum stress aging re-

sults. For example, although stresses as low as 20,000 to 25,000 pounds per square inch are effective for magnesium and aluminum alloys stresses far in excess of 50,000 to 60,000 pounds per square inch may be required for iron, nickel and cobalt alloys.

The "proportional limit" and "offset yield strengths" referred to in the description of the present invention are co-related properties derived from the stress-strain curves for standard tensile tests of metals and alloys. The first part of the stress-strain curve for those alloys whose recrystallization temperature is above room temperature, approximates a straight line and indicates that, throughout its range, the strain is directly proportional to the applied stress. The "proportional limit" is, therefore, the maximum applied stress for which strain remains directly proportional to stress. "Offset yield strengths" are determined by choosing a point on the strain-axis at some fixed (or chosen) displacement from the origin (for example, a strain of 1 or 2 thousandths of an inch per inch extension of the sample), and drawing a line from this point, parallel to the proportionality tangent at the proportional limit, to intersection with the stress-strain curve. Thus the 0.1% offset and 0.2% offset yield strengths are determined and are co-related to the proportional limit. Tests have shown (as is well-known) that the elastic limit may be as low as the proportional limit, but, in the vast majority of cases, elastic behavior extends above the proportional limit and may even extend beyond the 0.2% offset yield strength. Therefore, in the basic definition of stress-aging, the applied elastic stresses to effect maximum stress-aging effects are stated to be in the range of the proportional limit and may be as high as the 0.2% offset yield strength. Generally, loads in excess of the 0.2% offset yield strength cause measurable (true) permanent (plastic) deformation. Only the elastic portion of a plastic deformation load is effective in stress-aging and, since stress-aging is to be applied to stock (such as plate, rod, strip and wire) or shaped parts already finished to desired dimensions with close tolerances any further plastic deformation during stress-aging would be damaging or destructive to the material or parts thereof. Therefore, it is desirable that the stresses for stress-aging shall not be high enough to cause any damaging or destructive creep (permanent extension or distortion) during the stress-aging cycle.

The beneficial effects of my stress-aging process improve with increasing solute metal content. However, relatively small quantities of an alloy ingredient, whether an intentional addition or a normal impurity, may be very effective as in an alloy containing 1% cadmium and 99% copper. The ferrite matrix of plain carbon steels contain varying small quantities of carbon, manganese, silicon, etc. and such material has capacity for stress-aging. The same condition applies to commercial alloys all of which possess some degree of stress ageability. The metals, however, and particularly pure metals which lack any alloying ingredients, are so soft and characterized by such low elastic properties that stress-aging is far less effective than when applied to alloys. In general, therefore, my stress-aging process will be employed to best advantage only with alloys.

The stress-aging process may be carried out in various ways, for example formed springs of wire may be compressed, extended, or deflected and

the stressed spring aged while heated to the proper temperature by high frequency current or any other suitable means. Also, strip or wire may be stressed in tension and aged while heated by electrical resistance methods or the like. As applied to formed springs of wire, the process should not be confused with certain prior processes such as "stabilizing." If a sheet material of an alloy possessing good formability (such as aluminum alloys Alcoa 52S, 51ST, 53ST, 61ST, etc.) be cold formed into a desired shape for any spring-like use, repeated flexings in use will cause a re-alignment of the elastic strains (from cold forming) with a resultant warping of the part.

- 10 15 20 25 30 35 40 45 50
- If, after forming, the springing member be placed in a jig or form so that said member may be kept under slight elastic deflection in the desired operating direction, and said member (so restricted elastically) be heated at only slightly elevated temperatures (preferably at 150° F. or 65° C.) and re-cooled to room temperature under the same elastic restraint, the elastic strains will be re-aligned geometrically with the direction of spring operation during subsequent use of the part and no warping will occur during use. The standard tensile properties remain practically unaffected by this "stabilizing" treatment.

While this process of stabilizing is mechanically similar, in steps performed, to the steps

- 30 35 40 45 50
- employed in applicant's stress-aging process, both the applied stress in stabilizing and the temperature employed for stabilizing are too low to effect the marked increases in properties developed by applicant's stress-aging. In fact, one desired purpose of stabilizing is to retain as nearly as possible the original properties of the sheet material on which is predicated (by its engineering design) the operation in use of the stabilized part. Due consideration shows that stabilizing is thus distinctly different from applicant's stress-aging. For example, applicant's data show that stress-aging is ineffective for alloy 52S at temperatures below 125° C. (257° F.) and the benefits for stress-aging alloy 52S reach a maximum at 175° C. (347° F.). Moreover, the (elastic) stabilizing treatment is effective only for cold-worked (formed) parts, inclusive of pure metals, whereas applicant's stress-aging is shown to be effective for annealed alloys as well, but only for alloys containing effective amounts of solute metals (in solid solution).

Another example of stabilizing treatment is one applied to any spring acting part cut from cold-rolled sheet or strip. Thus coiled springs of cold-rolled brass, cold rolled steel, or of "bi-metal" (duplex strip of two alloys bonded together), etc., are coiled and tied in the coil shape (under slight elastic strain) and, so coiled, are stabilized at as low an elevated temperature as possible, depending on the alloy compositions involved.

- 55 60 65 70 75
- Strand-annealing is an established method of high efficiency and economy for continuously annealing or softening cold worked strip and wire. The strip or wire is drawn from loose coils or very free running reels or spools, pulled through the annealing furnace and rewound at the furnace exit. Since the purpose of strand annealing is to produce practically dead soft strip and wire for subsequent forming or further cold reduction, the strand-annealed product has very low strength properties. In annealing such soft materials, the stress employed in pulling the free running strip or wire through the furnace is kept as low as possible and far too low for any stress-

aging effects since practical annealing temperatures are considerably in excess of the recrystallization temperature and therefore too high for stress-aging. However, if the conventional strand annealing equipment is altered to maintain a desired high stress and proper relatively low aging temperatures, the desired stress-aging properties may be developed for the chosen material. This application of the invention differs from various means for controlling strand annealing temperatures which involve controlled plastic deformation and make use of the principle that each metal and alloy possess a definite tensile strength for each temperature so that tensile strength, may be used to measure temperature. It is well known, of course, that this relationship is true only for temperatures above the recrystallization temperature (or above the age-hardening temperature), as below these temperatures the tensile strength of any alloy will vary with the amount of preceding cold work (or degree of preceding precipitation-hardening). Thus the direct relationship of tensile strength to temperature applies only throughout the true hot-working range. In the hot-working range of temperatures, all metals and alloys are completely lacking in elasticity and hence possess no proportional limit, no elastic limit and none of the related offset yield strengths and any effective applied stress (below the tensile strength) is a plastic yield strength causing continuous yielding at rates varying with the amount of the applied stress and the temperature: the rate of yielding being approximately constant for a maintained constant stress and constant temperature. For strand-annealing and for strand-solution treatments (both at temperatures well above the respective recrystallization and age-hardening temperatures), wire or strip is passed continuously through a zone at the desired controlled elevated temperature. The length of this zone is necessarily related to the temperature and the time required at this temperature to achieve the necessary annealing or solution treatment for the specific alloy. When the correct relationship of high temperature, rate of travel of the strip or wire, and the length of the hot zone have been determined, it only remains in practice to control the temperature. Since, in the range of hot working temperatures, the tensile strength of the metal or alloy at the desired temperature is closely related to said temperature, a suitably lower stress may be applied to the strip or wire (by various mechanical means) as the strip or wire is passed through the established hot zone. Such a plastic yield strength, effective for the previously fixed length of the zone at temperature, will cause a specific amount of elongation and reduction in area of the strip and wire. Thus, under the given design and operating conditions for the hot zone, the rate of yield or amount of elongation (if measured continuously) or the reduced cross-section (of the strip or wire) can be used in various ways to effect temperature control (as by regulating fuel combustion or electric power for resistance heating). To employ such a method of temperature control, it is usually necessary to have the wire or strip at a suitable oversize previous to the heat treatment, depending upon the desired tolerances for the finished product.

It is obvious that processes employing either plastic deformation or temperatures resulting in recrystallization or over-aging (or solution) pre-

clude the use of applicant's process of stress aging. Moreover, the elastic stresses required for applicant's stress-aging process far exceed the plastic yield strengths employed in such processes, in fact, in most cases, would exceed the tensile strengths of the alloys at the operating temperatures of such processes.

While "stress-aging," the new treatment, consists of heating alloys under externally applied loads (or stresses) at temperatures not in excess of the recrystallization range, it is to be noted that none of the previously known heat treatments are conducted on materials under stress from external loads, for example, under tension. The following table summarizes pictorially the effects of these known treatments on physical properties as compared to the new treatment: "Stress-aging."

|                              | Elastic Properties | Tensile Strength | Per Cent Elong. | Electrical Conductivity |
|------------------------------|--------------------|------------------|-----------------|-------------------------|
| For Steels:                  |                    |                  |                 |                         |
| 25 1. Annealing.....         | D                  | D                | I               | I                       |
| 2. Hardening.....            | I                  | I                | D               | D                       |
| 3. Tempering.....            | D                  | D                | I               | I                       |
| For Precipitation Hardening: |                    |                  |                 |                         |
| 4. Solution.....             | D                  | D                | I               | D                       |
| 5. Aging.....                | I                  | I                | D               | I                       |
| For Solid Solutions:         |                    |                  |                 |                         |
| 30 6. Cold Work.....         | I                  | I                | D               | D                       |
| 7. Strain Relief.....        | C (D)              | C (D)            | C (I)           | I                       |
| 8. Annealing.....            | D                  | D                | I               | I                       |
| Stress-Aging (New).....      | I                  | I (C)            | I (C)           | I                       |

I=increase, D=decrease, C=constant. The use of parenthesis indicates alternative effect.

The effect of my stress-aging treatment can be made additive to the properties for cold worked solid solutions and also additive for aging of precipitation hardening. It also may be combined with or superimposed upon the tempering and annealing treatments for steels since the matrix for all steel microstructures consists of either alpha or gamma solid solutions based on the lattices of alpha or gamma iron.

The benefits of the stress-aging process as applied to each of eight commercial copper base alloys are hereinafter set forth in Tables Nos. 1 to 5 inclusive. The bars or test specimens were standard types, (a) threaded ends with 0.350" diameter reduced section in excess of 2" gage length and (b) threaded ends with 0.250" diameter reduced section in excess of the 2" gage length. Size (a) bars were used for all alloys except the initially higher strength 10% tin-Phosphor bronze for which size (b) was used for testing convenience. In each case a stress usually within the range of values between the proportional limit and a chosen yield strength relative to the specific alloy, was applied. While under such stress the alloys were heated for a desired length of time at effective temperatures and then cooled to room temperature under maintained stress. In each table the (A) lines indicate the property of the alloy in the stated commercial condition previous to stress-aging. All values in the tables are average for two or more bars each treated individually. The aging temperatures in all tables were chosen in the range of initial softening when the cold worked material is simply reheated as for standard strain relief and annealing. Heating periods of 4 and 75 20 hours were chosen arbitrarily.

TABLE 1

| Line | Stress-Aging        |      |      | Prop'l<br>Limit,<br>p. s. i. | 0.2% Yield<br>Strength | Tensile<br>Strength,<br>p. s. i. | Elong.,<br>Per Cent | Per Cent<br>R. A. |
|------|---------------------|------|------|------------------------------|------------------------|----------------------------------|---------------------|-------------------|
|      | Stress,<br>p. s. i. | Hrs. | ° C. |                              |                        |                                  |                     |                   |

## 70-30 BRASS: 36% COLD REDUCED

|    |        |    |     |        |        |        |      |    |
|----|--------|----|-----|--------|--------|--------|------|----|
| A1 | none   |    |     | 28,500 | 54,450 | 69,150 | 17   | 84 |
| 1  | 28,500 | 4  | 175 | 33,600 | 62,250 | 70,700 | 19.5 | 80 |
| 2  | 40,000 | 4  | 175 | 41,900 | 61,400 | 71,200 | 18   | 78 |
| 3  | 54,100 | 4  | 175 | 54,300 | 66,500 | 71,750 | 21   | 75 |
| 4  | 54,100 | 20 | 175 | 56,500 | 66,700 | 71,700 | 16   | 71 |
| 5  | 40,000 | 4  | 200 | 45,200 | 65,000 | 71,300 | 18   | 71 |
| 6  | 54,000 | 4  | 200 | 56,800 | 66,500 | 70,000 | 15   | 49 |
| 7  | 54,000 | 4  | 225 | 57,500 | 67,000 | 69,000 | 8    | 35 |

## 70-30 BRASS: 52% COLD REDUCED

|    |        |    |     |        |        |        |      |    |
|----|--------|----|-----|--------|--------|--------|------|----|
| A2 | none   |    |     | 28,400 | 69,800 | 86,750 | 13   | 80 |
| 8  | 28,400 | 4  | 175 | 39,200 | 74,450 | 87,250 | 11.5 | 75 |
| 9  | 40,000 | 4  | 175 | 49,000 | 80,000 | 88,500 | 11.5 | 73 |
| 10 | 54,100 | 4  | 175 | 60,400 | 85,400 | 88,700 | 12   | 73 |
| 11 | 69,800 | 20 | 175 | 71,000 | 86,800 | 88,750 | 10   | 71 |
| 12 | 40,000 | 4  | 200 | 55,200 | 87,400 | 90,000 | 11   | 71 |
| 13 | 54,000 | 4  | 200 | 60,200 | 87,400 | 89,800 | 11   | 71 |
| 14 | 54,000 | 4  | 225 | 68,400 | 88,000 | 88,500 | 10   | 61 |

TABLE 2

| Line | Stress-Aging        |      |      | Prop'l<br>Limit,<br>p. s. i. | 0.2% Yield<br>Strength | Tensile<br>Strength,<br>p. s. i. | Elong.,<br>Per Cent | Per Cent<br>R. A. |
|------|---------------------|------|------|------------------------------|------------------------|----------------------------------|---------------------|-------------------|
|      | Stress,<br>p. s. i. | Hrs. | ° C. |                              |                        |                                  |                     |                   |

## 85Cu-13.25Zn-1.75Pb: 35% COLD REDUCED

|    |        |   |     |                  |         |        |      |    |
|----|--------|---|-----|------------------|---------|--------|------|----|
| A3 | none   |   |     | 23,600           | 60,800  | 61,000 | 10   | 66 |
| 1  | 54,000 | 4 | 175 | 53,300           | 60,400  | 60,400 | 10   | 60 |
| 2  | 40,000 | 4 | 200 | 44,000           | 60,000  | 60,300 | 11   | 60 |
| 3  | 54,000 | 4 | 200 | 53,400           | 58,300  | 58,300 | 10   | 60 |
| 4  | 40,000 | 4 | 225 | 42,500           | 58,750  | 59,400 | 12   | 60 |
| 5  | 54,000 | 4 | 225 | broke in furnace | —3 hrs. |        | 7    | 48 |
| 6  | 40,000 | 4 | 250 | 44,100           | 57,800  | 58,350 | 12.5 | 60 |
| 7  | 40,000 | 4 | 275 | 42,850           | 53,700  | 55,650 | 10   | 48 |

## 85Cu-13.25Zn-1.75Pb: 50% COLD REDUCED

|    |        |   |     |        |        |        |     |    |
|----|--------|---|-----|--------|--------|--------|-----|----|
| A4 | none   |   |     | 27,350 | 75,000 | 76,200 | 8.5 | 66 |
| 8  | 54,000 | 4 | 175 | 60,000 | 75,000 | 75,700 | 9   | 60 |
| 9  | 40,000 | 4 | 200 | 51,900 | 74,800 | 75,500 | 9   | 60 |
| 10 | 63,500 | 4 | 200 | 60,900 | 74,000 | 75,000 | 10  | 60 |
| 11 | 40,000 | 4 | 225 | 49,600 | 72,350 | 74,500 | 10  | 60 |
| 12 | 63,500 | 4 | 225 | 63,100 | 71,900 | 72,750 | 9.5 | 48 |
| 13 | 40,000 | 4 | 250 | 48,400 | 71,500 | 72,600 | 9   | 60 |
| 14 | 40,000 | 4 | 275 | 50,800 | 69,300 | 71,250 | 10  | 55 |

TABLE 3

| Line | Stress-Aging        |      |      | Prop'l<br>Limit,<br>p. s. i. | 0.2% Yield<br>Strength | Tensile<br>Strength,<br>p. s. i. | Elong.,<br>Per Cent | Per Cent<br>R. A. |
|------|---------------------|------|------|------------------------------|------------------------|----------------------------------|---------------------|-------------------|
|      | Stress,<br>p. s. i. | Hrs. | ° C. |                              |                        |                                  |                     |                   |

## 6Sn-95Cu: 60% COLD REDUCED

|    |        |   |     |        |        |        |      |    |
|----|--------|---|-----|--------|--------|--------|------|----|
| A5 | none   |   |     | 39,400 | 86,500 | 87,550 | 14   | 76 |
| 1  | 39,400 | 4 | 175 | 56,200 | 82,050 | 86,550 | 17.5 | 76 |
| 2  | 45,000 | 4 | 175 | 58,350 | 83,300 | 86,300 | 15   | 76 |
| 3  | 75,000 | 4 | 175 | 75,200 | 86,000 | 86,800 | 17   | 76 |
| 4  | 45,000 | 4 | 200 | 56,250 | 80,350 | 86,400 | 18.7 | 76 |
| 5  | 75,000 | 4 | 200 | 73,250 | 82,000 | 87,000 | 20   | 76 |
| 6  | 45,000 | 4 | 225 | 58,600 | 78,300 | 85,800 | 22   | 76 |
| 7  | 75,000 | 4 | 225 | 74,500 | 80,200 | 85,050 | 19.5 | 76 |

## 10Sn-90Cu: 60% COLD REDUCED

|    |         |   |     |         |         |         |     |    |
|----|---------|---|-----|---------|---------|---------|-----|----|
| A6 | none    |   |     | 57,400  | 114,000 | 133,500 | 8.5 | 61 |
| 8  | 60,000  | 4 | 175 | 74,000  | 119,000 | 132,000 | 11  | 50 |
| 9  | 114,000 | 4 | 175 | 112,000 | 131,500 | 136,600 | 11  | 48 |
| 10 | 60,000  | 4 | 200 | 70,300  | 116,000 | 130,000 | 10  | 41 |
| 11 | 114,000 | 4 | 200 | 114,000 | 127,000 | 132,000 | 10  | 43 |
| 12 | 114,000 | 4 | 225 | 116,000 | 135,000 | 147,000 | 4   | 29 |

11  
TABLE 4

| Line | Stress Aging        |      |      | Prop'l<br>Limit,<br>p. s. i. | 0.2% Yield<br>Strength | Tensile<br>Strength,<br>p. s. i. | Elong.,<br>Per Cent | Per Cent<br>R. A. |
|------|---------------------|------|------|------------------------------|------------------------|----------------------------------|---------------------|-------------------|
|      | Stress,<br>p. s. i. | Hrs. | ° C. |                              |                        |                                  |                     |                   |

## 1Cd—99Cu:60% COLD REDUCED

|    |        |     |     |        |        |        |      |    |
|----|--------|-----|-----|--------|--------|--------|------|----|
| A7 | none   | --- | --- | 32,150 | 69,800 | 70,100 | 10   | 76 |
| 1  | 32,150 | 4   | 175 | 53,650 | 72,350 | 72,350 | 11   | 74 |
| 2  | 40,000 | 4   | 175 | 49,500 | 71,100 | 71,100 | 11   | 73 |
| 3  | 64,800 | 4   | 175 | 57,100 | 70,550 | 70,550 | 9.5  | 71 |
| 4  | 40,000 | 20  | 175 | 53,100 | 70,000 | 70,000 | 10   | 71 |
| 5  | 40,000 | 4   | 200 | 57,750 | 72,900 | 72,900 | 9.4  | 69 |
| 6  | 64,800 | 4   | 200 | 65,600 | 71,900 | 71,900 | 8.6  | 68 |
| 7  | 64,800 | 4   | 225 | 66,700 | 71,800 | 71,800 | 12.5 | 68 |

TABLE 5

| Line | Stress Aging        |      |      | Prop'l<br>Limit,<br>p. s. i. | 0.2% Yield<br>Strength | Tensile<br>Strength,<br>p. s. i. | Elong.,<br>Per Cent | Per Cent<br>R. A. |
|------|---------------------|------|------|------------------------------|------------------------|----------------------------------|---------------------|-------------------|
|      | Stress,<br>p. s. i. | Hrs. | ° C. |                              |                        |                                  |                     |                   |

## 8.3Al—2.9Fe—0.30Ni—88.5Cu:HOT EXTRUDED

|    |        |    |     |        |        |        |    |    |
|----|--------|----|-----|--------|--------|--------|----|----|
| A8 | none   | 4  | --- | 25,000 | 32,950 | 81,100 | 40 | 60 |
| 1  | 25,000 | 4  | 175 | 26,600 | 32,100 | 80,500 | 42 | 62 |
| 2  | 32,000 | 4  | 175 | 34,700 | 36,200 | 80,000 | 35 | 60 |
| 3  | 32,000 | 4  | 200 | 32,250 | 34,200 | 80,200 | 39 | 61 |
| 4  | 32,000 | 20 | 200 | 34,600 | 36,200 | 81,000 | 35 | 54 |
| 5  | 32,000 | 4  | 225 | 31,400 | 33,250 | 80,000 | 41 | 62 |
| 6  | 32,000 | 4  | 250 | 33,000 | 35,100 | 81,600 | 37 | 85 |

In Table #1 the proportional limit stress 28,500 per square inch applied to the 36% cold reduced alloy while aging for four hours at 175° C. gave increases of 18% for proportional limit, 14% for 0.2% yield strength, 2% for tensile strength, and 15% for elongation, whereas the yield strength stress 54,000 per square inch gave respective increases of 90%, 18%, 4% and 24%. A comparison of the results set forth on the line numbered 3 with those set forth on the line numbered 4 shows that four hours' aging gives about 96% of the increase in elastic properties (i. e. proportional limit, elastic limit and yield strength offset from 0.2% to 0.5% from the proportionality range of the stress strained curve) accomplished by 20 hours' aging.

In the test on 70-30 brass cold reduced 52% it will be noted that the increase in cold working provides a marked increase in yield strength and tensile strength with decreased elongation thereby permitting the use of higher stresses for stress-aging without damage from creep effects.

Table #2 sets forth the test results on hardware bronze, cold reduced 35% and 50%. As is normal for solid solution alloys the lower solute content (13.25% zinc) of hardware bronze as compared with 30% zinc in the 70-30 brass results in lower elastic properties and lower tensile strength. However, contrary to the usual effect of decreased solute metal content, decreasing the zinc content in copper zinc alloys actually results in a decrease in elongation. This increased basic rigidity causes a higher 0.2% yield strength in the lower zinc alloy, the yield strength being actually at or within the range of marked plastic deformation. This anomalous effect is apparently due to the unusual nature of the zinc atom, relative to the copper atom in the solid solution lattices. As indicated in lines numbered 4, 5, 6 and 7 of Table #2, the stress aging is surprisingly effective at those high temperatures which in the absence of stress actually exert an annealing effect causing a depreciation in ten-

sile properties from those given in line A3. In lines numbered 6 and 7 the test results show a slight lowering of tensile strength and yield strength from the stress aging maxima for 40,000 pounds per square inch (line numbered 2, Table 2) due to opposition of the annealing tendency at higher temperatures. A stress of 54,000 pounds per square inch actually caused embrittlement and fracture of the test bar during treatment at 225° C. The free lead in the hardware bronze alloy largely nullifies any stress aging effects on elongation and reduction of area so that in the absence of any embrittlement for excessive aging under stress these two properties remain relatively constant.

The 50% reduced alloy set forth in Table #2 stressages with surprising improvement in properties at higher temperatures that, in the absence of stress, would have an annealing effect. The presence of lead in hardware bronze tends to permit plastic flow once plastic deformation is well started. Hence, stress-aging has relatively small effect on elongation and reduction of area and the fractures retain the cup and cone type of break throughout the series.

Table #3 discloses the result of tests on two tin-Phosphor bronze alloys each 60% cold reduced and containing respectively 5 and 10% tin. The phosphorus content of each alloy is about 0.1% remaining after deoxidation. The stress aging effects for these alloys are of the same order as found for the other alloys of this series which lack phosphorus. The results obtained therefore are apparently not due to the small quantity of phosphorus present in the tin-Phosphor bronze alloys.

Table #4 sets forth the properties of a copper base alloy containing 1% cadmium and cold reduced 60%. Aging with an applied stress of 32,150 per square inch (the proportional limit of the plain cold worked material) for four hours at 175° C. resulted in an increase of 67% in proportional limit, 10% in the 0.1% yield strength

(64,800 per square inch) 3% in tensile strength and 10% in elongation.

Table #5 gives the properties of hot extruded aluminum bronze containing 8.3% aluminum, 2.9% iron, 0.30% nickel with the balance copper. This is a standard single phase commercial aluminum bronze composition. The alloy was hot extruded at temperatures well above the annealing temperature so that no cold work was effected. The tensile properties of the material untreated and as received are set forth in line 10 A8 and its microstructure shows the alloy to consist of a single solid solution phase free from any cold work.

The data for the alloys set forth in Tables 1 15 to 4 inclusive show that stresses in excess of

four hours at 175° C. gave effective increases of 32% in proportional limit and 12% in the 0.2% yield strength with practically constant tensile strength and a slight loss in elongation. The data of Table 5 indicates that hot worked or annealed solid solution phase-dominated alloys may be beneficially stress aged and that the cold worked condition, although helpful, is not a prerequisite for effective stress-aging. Previous cold work merely amplifies the degree of stress aging by permitting the use of much higher stresses during the aging periods.

For each of the eight alloys hereinbefore set forth the effects on electrical conductivity of two of the most effective stress-aging treatments are given in the following table:

TABLE 6  
*Effect of stress-aging treatments on electrical conductivity*

| Line | Alloy          | Elec. Cond'y., Per Cent | Stress-Aging     |      |      | Elec. Cond'y., Per Cent | Per Cent Increase |
|------|----------------|-------------------------|------------------|------|------|-------------------------|-------------------|
|      |                |                         | Stress, p. s. i. | Hrs. | ° C. |                         |                   |
| 1X   | 70-30 Brass    | 21.6                    | 40,000           | 4    | 200  | 27.5                    | 27                |
| 1Z   | 36% Cold Work  | 21.6                    | 54,000           | 4    | 200  | 27.8                    | 29                |
| 2X   | 70-30 Brass    | 21                      | 54,000           | 4    | 175  | 27.1                    | 30                |
| 2Z   | 52% Cold Work  | 21                      | 54,000           | 4    | 225  | 28.4                    | 35                |
| 3X   | H'dware Bronze | 29.6                    | 54,000           | 4    | 200  | 32.6                    | 10                |
| 3Z   | 35% Cold Work  | 29.6                    | 40,000           | 4    | 275  | 34.8                    | 19                |
| 4X   | H'dware Bronze | 29.2                    | 63,500           | 4    | 200  | 35.3                    | 21                |
| 4Z   | 50% Cold Work  | 29.2                    | 40,000           | 4    | 275  | 35.4                    | 21                |
| 5X   | 5 Sn P-Bronze  | 16.3                    | 75,000           | 4    | 175  | 20.7                    | 27                |
| 5Z   | 60% Cold Work  | 16.3                    | 45,000           | 4    | 225  | 21.7                    | 33                |
| 6X   | 10 Sn P-Bronze | 8.2                     | 114,000          | 4    | 175  | 10.4                    | 27                |
| 6Z   | 60% Cold Work  | 8.2                     | 114,000          | 4    | 225  | 10.5                    | 30                |
| 7X   | 1 Cd-99 Cu     | 60.4                    | 40,000           | 4    | 200  | 83.0                    | 20                |
| 7Z   | 60% Cold Work  | 69.4                    | 64,000           | 4    | 200  | 83.1                    | 20                |
| 8X   | Al-Bronze      | 11.9                    | 32,000           | 4    | 200  | 12.1                    | 2                 |
| 8Z   | No Cold Work   | 11.9                    | 32,000           | 20   | 200  | 12.1                    | 2                 |

about 30,000 pounds per square inch produce the great improvement that can be effected by stress aging. In the annealed condition all of the 45 copper base alloys set forth in Tables 1 to 4 inclusive lack the necessary strength to support the stresses required for the most effective stress-aging. The properties of aluminum bronze with a proportional limit of 25,000 pounds per square inch indicates that the mere addition of a cold worked structure is not a requirement for stress-aging other than for initial strengthening purposes. However, due to its relatively high elongation (40% in the hot extruded or annealed condition) the 0.2% yield strength of about 33,000 pounds per square inch is much lower than for any of the cold worked alloys set forth in Tables 1 to 4 inclusive. Thus, only a very narrow range of aging stresses, between 25,000 60 pounds per square inch and 33,000 pounds per square inch, can be expected to be really effective for stress aging this aluminum bronze alloy since higher loads would cause destructive plastic deformation within the time required for effective stress-aging at any useful temperature. This aluminum bronze will not support a stress of 32,000 pounds per square inch for much more than four hours at 200° C. or as long as four hours at 250° C.

It will be noted that the proportional limit aging stress of 25,000 pounds per square inch for four hours at 175° C. gave negligible increases in proportional limit and elongation. Aging under a stress of 32,000 pounds per square inch for

55 The data in this table indicates, (1) that stress aging increases electrical conductivity in all cases, (2) that for the same aging treatment (time at temperature) higher stresses result in higher conductivities, (3) that for the same stress, higher aging temperatures yield higher conductivities, (4) that given a minimum effective stress, (above the elastic limits of the untreated materials) increase in aging temperature is more effective in degree than increase in stress, (5) that with sufficiently effective stress-aging, the resulting electrical conductivities may even exceed that of the annealed single-phase solid solution alloy, as indicated in the following items:

- (a) Electrical conductivity of annealed "70-30" brass is 27% of that of pure copper. The resulting conductivities for 1X, 1Z, 2X and 2Z are slightly in excess of 27%.
- (b) Electric conductivity of annealed 5Sn bronze is 17%. Stress aged bars 5X and 5Z have conductivities about 20 to 30% in excess of 17%.
- (c) Electrical conductivity of annealed 10Sn bronze is about 9%. Stress aged bars 6X and 6Z have conductivities about 15% in excess of 9%.

70 The combination of increased electrical conductivity with the observed increases in tensile properties is believed to be unique for the "stress-aging" treatment.

75 In addition to copper-base alloys (Class A),

other solid solution alloys such as the following can be processed by the present invention:

*Class B.*—Stainless steel

*Class C.*—Solid solution Fe-base alloys

*Class D.*—Precipitation-hardened Fe-base alloy

*Class E.*—Solid solution Al-base alloys

*Class F.*—Precipitation-hardened (or heat-treated) Al-base alloys.

It is to be understood of course that this classification is wholly arbitrary and non-limiting.

#### CLASS B.—STAINLESS STEEL

The material treated had the following typical analysis: 18.33% Cr—9.32% Ni—0.10% C—0.91% Mn—0.41% Si and the balance Fe. The stock was  $\frac{1}{2}$ " diameter hard drawn rod, finished with 38% cold reduction, giving about the maximum strength properties for rod of this size.

Reference to Tables 7 and 7A will give the results of stress-aging the stainless steel. Line 1 in both tables gives the tensile properties of the plain cold worked alloy (as received). Stainless steel of this type is a rather complicated alloy (not an "un-heat-treatable" single solid-solution phase as is alpha brass). Stainless steel can be made austenitic at room temperature by quenching it from above 1000° C. Subsequent cold work tends to transform the Austenite into alpha ferrite. Also reheating in the range of 400–600° C. causes precipitation of carbides if even 0.1% C is present (unless the alloy is stabilized by converting the carbon into insoluble carbides, such as those of tantalum or columbium).

stressed by line 2, Table 7. Line 3 shows the cold-work strengthening of stainless steel at room temperature caused by a stress of 90,000 p. s. i., just above the elastic limit. Line 4 shows the 5 strengthening at room temperature by a stress of 150,000 p. s. i., well into the plastic range of this alloy.

Plastic deformation of an alloy at temperatures below its recrystallization range will cause cold work strengthening but this strengthening diminishes rapidly with increase in temperature of the cold-working. Thus the cold-work strengthening of alloys at temperatures just below their recrystallization range is greatly less than the 15 strengthening by equal cold plastic deformation at room temperature, when room temperature is effectively below the recrystallization range. Thus the strengthening effect of 90,000 p. s. i. stress in the aging range of 400 to 600° C. is very 20 much less than at room temperature. Therefore, comparison of line 3, Table 7, with lines 5 to 14 shows that the stress-aging effects on properties (proportional limit is of special importance for engineering design) of stainless steel cannot at 25 all be explained by any cold-working interpretation. In fact, the marked strengthening effect of 90,000 p. s. i. stress-aging for only 15 minutes at 400° C. (line 5) would rule out any effective plastic flow for such a short time as 4 hrs. at 30 these temperatures. There is no measurable creep until the stress-aging temperatures exceed 500° C., whereupon the annealing effect begins to overcome the stress-age-strengthening effect.

TABLE 7  
Properties of stress-aged 18 Cr-9 Ni stainless steel (cold worked 38%)

| Line | Stress-Aging     |         |     | Prop'l Limit         | 0.2% Offset Yield Strength | Tensile Strength | Elong., Per Cent | Per Cent R. A. |
|------|------------------|---------|-----|----------------------|----------------------------|------------------|------------------|----------------|
|      | Stress, p. s. i. | Hrs.    | °C. |                      |                            |                  |                  |                |
| 1    | none             | —       | —   | 72,300               | 178,500                    | 193,200          | 7.5              | 37             |
| 2    | 72,300           | 4       | 25  | 72,200               | 178,600                    | 193,800          | 7.5              | 37             |
| 3    | 90,000           | 4       | 25  | 105,000              | 174,600                    | 194,200          | 7.0              | 36             |
| 4    | 150,000          | 4       | 25  | 120,000              | 176,600                    | 192,900          | 2.0              | 30             |
| 5    | 90,000           | 15 min. | 400 | 133,400              | 188,900                    | 202,200          | 8.5              | 36             |
| 6    | 90,000           | 30 min. | 400 | 138,700              | 187,700                    | 202,600          | 8.5              | 38             |
| 7    | 90,000           | 45 min. | 400 | 139,700              | 188,200                    | 201,900          | 8.5              | 38             |
| 8    | 90,000           | 1       | 400 | 138,300              | 188,600                    | 202,600          | 8.5              | 38             |
| 9    | 90,000           | 2       | 400 | 140,000              | 188,100                    | 203,100          | 8.5              | 38             |
| 10   | 90,000           | 4       | 400 | 142,000              | 191,000                    | 235,400          | 8.5              | 39             |
| 11   | 90,000           | 4       | 450 | 136,000              | 197,600                    | 204,000          | 8.5              | 42             |
| 12   | 90,000           | 4       | 500 | 134,000              | 193,000                    | 197,300          | 8.5              | 40             |
| 13   | 90,000           | 4       | 550 | 128,000              | 170,000                    | 182,000          | 6.0              | 46             |
| 14   | 90,000           | 4       | 600 | 114,000              | 159,000                    | 176,500          | 13.5             | 42             |
| 15   | 150,000          | 4       | 400 | 154,000              | 206,000                    | 208,800          | 8.5              | 42             |
| 16   | 150,000          | 4       | 450 | Bar broke in furnace |                            |                  |                  |                |
| 17   | 150,000          | 4       | 500 | Bar broke in furnace |                            |                  |                  |                |

TABLE 7A  
Properties of plain aged 18 Cr-9 Ni stainless steel (cold worked 38%)

| Line | Plain Aging (No applied stress) |     | Prop'l Limit | 0.2% Offset Yield Strength | Tensile Strength | Elong., Per Cent | Per Cent R. A. |
|------|---------------------------------|-----|--------------|----------------------------|------------------|------------------|----------------|
|      | Hrs.                            | °C. |              |                            |                  |                  |                |
| 1    | Un-Aged                         | —   | 72,300       | 178,500                    | 193,200          | 7.5              | 37             |
| 2    | 4                               | 400 | 96,500       | 180,000                    | 197,000          | 7.5              | 63             |
| 3    | 4                               | 450 | 93,000       | 181,000                    | 195,000          | 7.5              | 60             |
| 4    | 4                               | 500 | 92,800       | 170,000                    | 183,000          | 6.0              | 61             |
| 5    | 4                               | 550 | 88,000       | 171,000                    | 184,000          | 7.5              | 62             |

As is well known, stressing an alloy below its elastic limit for relatively short times (so that creep remains unmeasurable) will not affect its previous physical properties. The proportional limit is below the elastic limit. This is demon-

and the stress-aged properties begin to decline (or over-age).

Table 7A shows the effects on tensile properties of aging the same alloy at the same temperatures (as for stress-aging) but in the absence

of any externally applied stress. Lines 2 to 5 of Table 7A show relatively small increases in strength properties due to the carbide precipitation effect previously described. This effect is distinctly minor as compared to the effects of stress-aging stainless steel. It is also to be noted that the effects of plain aging on the elongation and reduction of area are markedly different from the effects of stress-aging and not nearly so beneficial.

The maximum effect of 90,000 p. s. i. stress-aging of stainless steel results for the treatment shown in line 10, Table 7: 4 hours at 400° C. However, 15 minutes stress-aging at 400° C. gives better than 90% of the improvement effected by 4 hours.

Stress-aging with 150,000 p. s. i. is effective on properties but destructive creep at this stress occurs at 400° C. and stress-aging at such higher stresses is impossible at higher temperatures as the alloy fractures during the treatment (shown by lines 15, 16, 17, Table 7).

#### CLASS C.—SOLID SOLUTION Fe-BASE ALLOYS

These are solid-solution alloys that are not amenable to heat treatment except for annealing to remove all effect of cold work properties and structure.

The compositions of these 3 representative alloys were as follows:

A. 36Ni—0.10C—0.45Mn—0.20Si—0.03P—0.03S—bal. Fe.

B. 19.5Ni—2.25Cr—1.0Mn—0.20Si—0.03P—0.03S—bal. Fe.

C. 18Ni—11Cr—0.25C—0.40Mn—0.15Si—0.03P—0.03S—bal. Fe.

10 The recrystallization and actual annealing temperatures are as follows:

|     | Recrystallization Temperature | Annealing Temperature |
|-----|-------------------------------|-----------------------|
|     | ° C.                          | ° C.                  |
| (A) | 705                           | 735                   |
| (B) | 815                           | 1,040                 |
| (C) | 815                           | 1,040                 |

Since these alloys are in the annealed condition, simply reheating them to such lower temperatures as were employed for subsequent stress-aging would have no measurable effect on their annealed properties. The properties of these alloys, in the initial annealed state, are given respectively in lines 1, 7 and 13 in Table 8.

TABLE 8  
*Properties of 3 annealed Fe-Base solid-solution alloys, Effect of Stress-aging*

| Line                                       | Stress-Aging Treatment |      |      | Creep <sup>1</sup> | Prop'l Limit | 0.2% Offset Yield Strength | Tensile Strength | Elong., Per Cent | Per Cent R. A. |
|--------------------------------------------|------------------------|------|------|--------------------|--------------|----------------------------|------------------|------------------|----------------|
|                                            | Stress, p. s. i.       | Hrs. | ° C. |                    |              |                            |                  |                  |                |
| <b>A. 36% Ni—64% Fe ALLOY, ANNEALED</b>    |                        |      |      |                    |              |                            |                  |                  |                |
| 1                                          | None                   |      |      |                    | 25,000       | 40,000                     | 70,000           | 35               | 65             |
| 2                                          | 25,000                 | 4    | 400  | 0                  | 45,800       | 68,000                     | 84,500           | 21               | 81             |
| 3                                          | 40,000                 | 4    | 400  | 0                  | 56,500       | 69,500                     | 84,500           | 21               | 81             |
| 4                                          | 40,000                 | 20   | 400  | .001               | 57,200       | 65,400                     | 81,200           | 20               | 80             |
| 5                                          | 25,000                 | 4    | 500  | .005               | 47,800       | 59,800                     | 80,700           | 25               | 78             |
| 6                                          | 40,000                 | 4    | 500  | .300               | 52,600       | 68,800                     | 84,800           | 16               | 77             |
| <b>B. 19Ni—2Cr—79% Fe ALLOY, ANNEALED</b>  |                        |      |      |                    |              |                            |                  |                  |                |
| 7                                          | None                   |      |      |                    | 30,000       | 45,000                     | 85,000           | 40               | 60             |
| 8                                          | 30,000                 | 4    | 400  | 0                  | 68,500       | 84,000                     | 122,200          | 32               | 71             |
| 9                                          | 45,000                 | 4    | 400  | 0                  | 75,400       | 85,600                     | 121,800          | 29               | 67             |
| 10                                         | 45,000                 | 20   | 400  | 0                  | 69,200       | 80,000                     | 116,000          | 40               | 73             |
| 11                                         | 30,000                 | 4    | 600  | 0                  | 62,200       | 82,500                     | 120,000          | 30               | 69             |
| 12                                         | 40,000                 | 4    | 500  | 0                  | 65,800       | 75,700                     | 117,500          | 38               | 69             |
| <b>C. 18Ni—11Cr—71% Fe ALLOY, ANNEALED</b> |                        |      |      |                    |              |                            |                  |                  |                |
| 13                                         | None                   |      |      |                    | 25,000       | 40,000                     | 85,000           | 42               | 55             |
| 14                                         | 25,000                 | 4    | 400  | 0                  | 59,900       | 86,750                     | 110,000          | 25               | 65             |
| 15                                         | 40,000                 | 4    | 400  | 0                  | 74,300       | 101,500                    | 120,000          | 36               | 66             |
| 16                                         | 65,000                 | 20   | 400  | 0                  | 89,200       | 101,500                    | 117,000          | 20               | 60             |
| 17                                         | 25,000                 | 4    | 600  | 0                  | 42,700       | 48,300                     | 99,800           | 22               | 63             |
| 18                                         | 40,000                 | 4    | 500  | 0                  | 72,800       | 99,500                     | 120,000          | 21               | 62             |

<sup>1</sup> Creep, during stress-aging, reported as inches per inch length.

Three alloys of this type were stress-aged at temperatures below recrystallization, the alloys being in the annealed state previous to stress-aging. Whereas the copper-base alloys must be cold worked in order to sustain effective loads for stress-aging, such iron-base alloys as these are inherently strong enough in the annealed state to be very effectively stress-aged. This is mentioned in order to again emphasize the fact that cold work is not an inherent requirement for stress-aging, merely that cold work strengthens the alloy previous to stress-aging, thereby permitting more effective subsequent stress-aging.

These alloys stress-aged so effectively (and quickly) that, in only one instance, (line 6, Table 8), did destructive creep take place during the stress-aging period of 4 hours, even though stresses considerably above the proportional limit were also employed (note especially line 16, Table 8).

70 The outstanding effect and improvement in physical properties is obvious. An extreme case is to be noted for the alloy C wherein stress-aging under 65,000 p. s. i. for 20 hours at 400° C. increased the proportional limit for this alloy from 25,000 p. s. i. in the annealed state to 89,200 p. s. i.,

even higher than the tensile strength as annealed (85,000 p. s. i.).

The maximum stress-aging effects for these alloys are given respectively in lines 3, 9 and 16 (15 is more practical) of Table 8. These maximum stress-aged properties markedly exceed the properties for the same alloys when cold-worked 50% although the stress-aging treatment involved no measurable plastic deformation. As is the case with the copper-base alloys, these Fe-base alloys can be similarly improved by stress-aging subsequent to cold-working.

CLASS D.—PRECIPITATION-HARDENED Fe-BASE ALLOY

"Ni-Span-C" has the following composition: 42% Ni—5.5Cr—2.5Ti—0.1 carbon—bal. Fe, containing usual minor impurities. Due to its titanium content (together with Ni), this alloy can be markedly improved by an inherent precipitation reaction. Its complete precipitation heat treatment is as follows: (a) solution treatment: heat to 950° C. and quench, (b) then age 2 to 4 hours at 675° C. The precipitation-hardening effect of aging the solution-treated alloy does not appreciably change the properties until the aging temperature exceeds 500° C. This permits stress-aging tests of the solution-treated alloy in the range of 400–500° C. without appreciable overlapping of inherent precipitation reaction. In Table 9, the properties of the solution-treated alloy are given in line 1. Lines 2 and 3 show that this alloy yields stress-aging effects similar to those of the 3 annealed Fe-base alloys cited above (Class C).

essentially inert at temperatures below and about at the critical aging temperature.

Line 4 of Table 9 gives the tensile properties for "Ni-Span C" fully age-hardened. Lines 5, 6 and 7 show that these properties can be markedly improved by subsequent stress-aging. The preferred stress-aging treatment is that of line 5.

CLASS E.—SOLID SOLUTION Al-BASE ALLOYS

Two non-heat-treatable (except for annealing or strain relief treatments) Al-base alloys are known commercially as 2S and 52S. Their compositions are as follows:

15 2S.—From 1 to 2% impurities, chiefly Fe and Si.  
52S.—2.5% Mg—0.25% Cr—ordinary impurities.

20 Stronger lattice binding within the crystal structures of metals and alloys results in higher melting temperatures, since the greater thermal agitation at higher temperatures is required to break the inter-atomic linkage and cause melting. Thus alloys with higher melting ranges will require greater applied stresses for maximum stress-aging results. Relative to the results cited herein for stress-aging, stresses as low as 20–25,000 p. s. i. may be effective for alloys of Mg or of Al whereas alloys of Fe, Ni, or Co will usually require stresses of 50–60,000 p. s. i. with Cu-base alloys requiring intermediate minimum load stresses. Further, stress-aging effects are more pronounced for higher solute metal solid solutions.

30 Al-alloys 2S and 52S were tested in their respective  $\frac{1}{2}$  hard and  $\frac{1}{4}$  hard cold-worked con-

TABLE 9

Properties of "Ni-Span C" precipitation-harden-  
ing alloy, in its solution-treated and its precip-  
itation-aged conditions, effect of stress-aging

| Line                   | Stress-Age Treat-<br>ment |      |      | Creep <sup>1</sup> | Prop'l<br>Limit | 0.2%<br>Offset<br>Yield<br>Strength | Tensile<br>Strength | Elong.,<br>Per Cent | Per Cent<br>R. A. |
|------------------------|---------------------------|------|------|--------------------|-----------------|-------------------------------------|---------------------|---------------------|-------------------|
|                        | Stress,<br>p. s. i.       | Hrs. | ° C. |                    |                 |                                     |                     |                     |                   |
| PLAIN SOLUTION-TREATED |                           |      |      |                    |                 |                                     |                     |                     |                   |
| 1.                     | None                      |      |      |                    | 15,000          | 35,000                              | 90,000              | 40                  | 60                |
| 2.                     | 35,000                    | 4    | 400  | 0                  | 50,000          | 51,000                              | 93,000              | 38                  | 66                |
| 3.                     | 35,000                    | 4    | 500  | 0                  | 52,200          | 54,200                              | 99,800              | 39                  | 66                |
| PRECIPITATION-AGED     |                           |      |      |                    |                 |                                     |                     |                     |                   |
| 4.                     | None                      |      |      |                    | 65,000          | 115,000                             | 165,000             | 16                  | 30                |
| 5.                     | 90,000                    | 4    | 400  | 0                  | 99,000          | 123,000                             | 164,000             | 17                  | 45                |
| 6.                     | 115,000                   | 4    | 400  | .08                | 131,500         | 135,000                             | 164,500             | 15                  | 50                |
| 7.                     | 65,000                    | 4    | 500  | 0                  | 94,200          | 123,000                             | 164,000             | 16                  | 40                |

<sup>1</sup> Creep, during stress-aging, reported as inches per inch length.

For alloys that can be precipitation-hardened to maximum properties, subsequent aging at temperatures below (and at) that of the critical heat-treatment will effect no further increase in strength properties. In fact, the only effect for extremely long periods of heating at such temperatures will be a tendency to over-age with marked decreases in strength properties. It is obvious therefore that, if stress-aging is superimposed upon a precipitation-hardened alloy, any improvement in strength properties will be due to stress-aging effects in the matrix solid solution, the previously precipitated phase remaining

diluted (respectively 21% and 11% cold reduction). Their properties in the cold worked condition are given respectively in lines 1 and 7 of Table 10. Their proportional limits and 0.2% offset yield strengths are so low (as are also their solute metal contents) that it is to be expected that stress-aging improvements of their properties would, at best, be relatively small. The results of stress aging treatments, as given in Table 10 bear this out, although it is to be noted that their proportional limits can be increased in the range of 20 to 30% (lines 2, 3, and 9, 11 of Table 10).

TABLE 10  
Effect of stress-aging on two cold worked, solid solution, aluminum alloys

| Line                         | Stress-Age Treatment |      |      | Creep, Per Cent | Prop'l Limit | 0.2% Off-set Yield Strength | Tensile Strength | Elong., Per Cent |
|------------------------------|----------------------|------|------|-----------------|--------------|-----------------------------|------------------|------------------|
|                              | Stress, p. s. i.     | Hrs. | ° C. |                 |              |                             |                  |                  |
| COLD WORKED Al-ALLOY 2S ½ H  |                      |      |      |                 |              |                             |                  |                  |
| 1                            | None                 | 4    |      | 0               | 11,000       | 17,850                      | 20,000           | 20               |
| 2                            | 11,000               | 4    | 100  | 0               | 13,600       | 17,700                      | 19,900           | 19               |
| 3                            | 11,000               | 4    | 125  | 0               | 13,600       | 17,700                      | 19,600           | 21               |
| 4                            | 10,500               | 4    | 150  | 0               | 12,400       | 17,600                      | 19,500           | 19               |
| 5                            | 7,750                | 4    | 175  | 0               | 12,900       | 17,350                      | 19,200           | 19               |
| 6                            | 7,750                | 4    | 200  | 3               | 12,000       | 14,900                      | 17,600           | 21               |
| COLD WORKED Al-ALLOY 52S ¼ H |                      |      |      |                 |              |                             |                  |                  |
| 7                            | None                 | 4    |      | 0               | 17,500       | 26,000                      | 32,800           | 16               |
| 8                            | 17,500               | 4    | 100  | 0               | 17,700       | 24,600                      | 32,200           | 19               |
| 9                            | 26,000               | 4    | 100  | 0               | 25,200       | 26,800                      | 32,000           | 19               |
| 10                           | 17,500               | 4    | 125  | 0               | 18,700       | 23,600                      | 31,700           | 20               |
| 11                           | 26,000               | 4    | 125  | 2               | 22,400       | 26,200                      | 31,700           | 21               |
| 12                           | 17,500               | 4    | 150  | 0               | 19,200       | 22,900                      | 32,200           | 20               |
| 13                           | 17,500               | 4    | 175  | 0               | 19,400       | 22,900                      | 33,600           | 22               |
| 14                           | 17,500               | 4    | 200  | 1               | 18,200       | 22,300                      | 32,200           | 19               |

As the heat-treated Al-alloys possess considerably higher strength properties, improvements of 20 to 30% in their elastic properties would be more valuable from a commercial standpoint.

CLASS F.—HEAT-TREATED Al-BASE ALLOYS

| Alloy | Composition             | Stress Aging Table |
|-------|-------------------------|--------------------|
| 14ST  | 4.4Cu—0.8Si—0.8Mn—0.4Mg | 11                 |
| 17ST  | 4.0Cu—0.5Mn—0.5Mg       | 12                 |
| 18ST  | 4.0Cu—0.5Mg—0.5Ni       | 13                 |
| 24ST  | 4.5Cu—0.6Mn—1.5Mg       | 14                 |
| 75ST  | 1.6Cu—0.2Mn—2.5Mg—5.6Zn | 15                 |

For alloys that are age-hardened to maximum properties, subsequent aging at temperatures below (and at) that of the original aging treatment will effect no further increase in strength properties. In fact, the only effect for even extremely long periods of heating at such temperatures will be a tendency to over-age with marked decreases in strength properties. It is obvious that, if stress-aging is superimposed upon a precipitation-hardened alloy, any increase in strength properties will be due to stress-aging effects in the matrix solid solution, the quantity of the previously precipitated phase remaining unaffected but added to by further precipitation effects induced by the new stress-aging treatment. Thus the matrix (parent) solid solution phase of the fully precipitation-hardened alloys should be susceptible to subsequent stress-aging treatment just as in the case of "unheat-treatable" solid-solution alloys (alpha brass for example). However, since the matrix solid-solution phase of fully age-hardened alloys has already been effectively depleted of solute metal content by the normal precipitation reaction, the effect of subsequent stress-aging on properties

will be less in degree than for the single phase solid-solution alloys, such as alpha brass, (an improvement of about 30-50% for the proportional limit as compared to 100-150% in the case of the such alloys as alpha brass). Thus, for the presently cited heat-treatable Al alloys, the solute metal content of the matrix solid solution phases of the fully age-hardened alloys is higher than for "solid-solution" alloys 2S and 52S and yet considerably lower than for such alloys as alpha brasses and bronzes. Also, the heat-treatable Al alloys will withstand much higher load stresses during stress-aging than do the solid solution Al alloys 2S and 52S.

Each of the 5 representative heat-treatable Al alloys was given its standard complete heat-treatment for "maximum" known strength properties. Samples of each heat-treated alloy were then stress-aged at stresses including values equal to the room temperature proportional limits and 0.2% offset yield strengths for the specific (heat-treated) alloy for 4 hrs. at each of a succession of temperatures ranging from 100° C. to above the characteristic aging temperature for each specific alloy. The standard period of 4 hours for aging under the stated applied loads was arbitrarily chosen since it has been determined that 15 minutes of stress-aging generally yields from 50 to 80% of the effect of 4 hours stress-aging and 4 hours aging generally yields 90% or more of the effect of 20 hours of stress-aging. In industry, 4 hours for stress-aging would appear to be about the maximum practical time that would be allowed for this treatment and, for maximum economic efficiency, a 15 minute stress-aging period should be used whenever it is sufficiently efficacious.

Brief comments on each of the 5 representative heat-treatable Al-alloys follow:

TABLE 11  
Properties of aluminum alloy 14ST after stress-aging

| Line | Stress-Age Treatment |      |      | Creep, Per Cent | Prop'l Limit | 0.2% Off-set Yield Strength | Tensile Strength | Elong., Per Cent |
|------|----------------------|------|------|-----------------|--------------|-----------------------------|------------------|------------------|
|      | Stress, p. s. i.     | Hrs. | ° C. |                 |              |                             |                  |                  |
| 1    | None                 | 4    |      | 0               | 43,800       | 55,300                      | 65,700           | 13               |
| 2    | 44,000               | 4    | 100  | 0               | 43,300       | 55,000                      | 65,200           | 13               |
| 3    | 55,000               | 4    | 100  | 0               | 51,700       | 57,700                      | 64,200           | 13               |
| 4    | 44,000               | 4    | 125  | 0               | 45,500       | 54,800                      | 64,300           | 13               |
| 5    | 55,000               | 4    | 125  | 1               | 51,000       | 57,400                      | 64,200           | 15               |
| 6    | 44,000               | 4    | 150  | 0               | 46,200       | 55,800                      | 65,800           | 13               |
| 7    | 44,000               | 4    | 175  | 0               | 47,500       | 57,400                      | 66,200           | 13               |
| 8    | 40,000               | 4    | 200  | 0               | 46,400       | 57,400                      | 65,800           | 10               |
| 9    | 30,000               | 4    | 225  | 0               | 43,400       | 51,500                      | 59,500           | 8                |
| 10   | 25,000               | 4    | 250  | 0               | 34,800       | 46,400                      | 56,000           | 7                |

Line 1 gives the tensile properties for alloy 14ST in its normally age-hardened condition. Line 3 gives the preferred stress-aging treatment for maximum elastic (engineeringly useful) properties without destructive (practically measurable) creep. By line 3 stress-aging treatment, the proportional limit is increased by about 20% with no loss in elongation. Plain prolonged aging at 150° C. (in the absence of any applied stress) results in overaging (or annealing) with properties as follows: 28,000 proportional limit, 39,000 0.2% offset yield strength, 43,000 tensile strength and 16% elongation. These properties are to be compared with line 6 for 150° C. stress-aging. Plain prolonged aging at 250° C. results in the following properties: no proportional limit, 8,000 0.2% offset yield strength, 10,000 tensile strength and 50% elongation. These properties should be compared with the 250° C. stress-aging of line 10.

Line 1 gives the tensile properties for alloy 17ST in its normally heat-treated condition. Line 10 gives the preferred stress-aging treatment for maximum elastic properties without destructive creep. By line 10 stress-aging treatment, the proportional limit is increased by 40%, and the 0.2% offset yield strength is increased by 20%. Even though the elongation for this treatment decreased to 13% this value still represents excellent ductility for engineering use. An alternative beneficial stress-aging treatment is that of line 3. It will be noted that for alloy 17ST (and several others of this group) stress-aging under the proportional limit stress with increasing stress-aging temperature causes initial increases in elastic properties, then passes through a minimum value to continue to a second and considerably greater maximum effect.

TABLE 13

*Properties of aluminum alloy 18ST after stress-aging*

| Line | Stress-Age Treatment |      |      | Creep, Per Cent | Prop'l Limit | 0.2% Off-set Yield Strength | Tensile Strength | Elong., Per Cent |
|------|----------------------|------|------|-----------------|--------------|-----------------------------|------------------|------------------|
|      | Stress, p. s. i.     | Hrs. | ° C. |                 |              |                             |                  |                  |
| 1    | None                 |      |      |                 | 36,050       | 47,500                      | 59,100           | 12               |
| 2    | 36,000               | 4    | 100  | 0               | 39,100       | 51,000                      | 62,200           | 16               |
| 3    | 47,500               | 4    | 100  | 0               | 45,800       | 51,300                      | 59,200           | 14               |
| 4    | 36,000               | 4    | 125  | 0               | 39,000       | 50,700                      | 61,200           | 12               |
| 5    | 47,500               | 4    | 125  | 0               | 45,700       | 52,800                      | 62,200           | 12               |
| 6    | 35,000               | 4    | 150  | 0               | 38,600       | 49,000                      | 59,500           | 12               |
| 7    | 47,500               | 4    | 150  | 2               | 45,200       | 52,700                      | 58,500           | 12               |
| 8    | 36,000               | 4    | 175  | 0               | 38,300       | 49,100                      | 60,000           | 12               |
| 9    | 29,000               | 4    | 200  | 0               | 36,200       | 47,800                      | 58,800           | 10               |
| 10   | 28,800               | 4    | 225  | 0               | 31,000       | 45,800                      | 54,500           | 12               |
| 11   | 23,000               | 4    | 250  | 0               | 30,200       | 42,200                      | 50,100           | 10               |

These comparisons show that, not only does stress-aging yield improved properties but that stress-aging opposes the normal overaging or annealing reaction until the temperature is high enough (in excess of the normal critical aging temperature of the standard heat-treatment) for the normal annealing (over-aging) tendency to completely overcome the stress-induced (stress) aging reaction. Such plain-aging vs. stress-aging comparisons hold for all 5 of these representative heat treated Al-alloys.

Line 1 gives the tensile properties for alloy 18ST in its normally heat-treated condition. Lines 3 and 5 give two, practically equivalent, preferred stress-aging treatments for maximum elastic properties (unaccompanied by destructive creep). The proportional limit is increased by about 30%, and the yield strength by about 8% with elongation constant or slightly increased.

TABLE 12

*Properties of aluminum alloy 17ST after stress-aging*

| Line | Stress-Age Treatment |      |      | Creep, Per Cent | Prop'l Limit | 0.2% Off-set Yield Strength | Tensile Strength | Elong., Per Cent |
|------|----------------------|------|------|-----------------|--------------|-----------------------------|------------------|------------------|
|      | Stress, p. s. i.     | Hrs. | ° C. |                 |              |                             |                  |                  |
| 1    | None                 |      |      |                 | 36,500       | 48,000                      | 65,000           | 24               |
| 2    | 36,000               | 4    | 100  | 0               | 38,500       | 46,000                      | 65,200           | 25               |
| 3    | 48,000               | 4    | 100  | 0               | 46,700       | 48,700                      | 64,800           | 25               |
| 4    | 36,000               | 4    | 125  | 0               | 35,000       | 41,200                      | 63,200           | 25               |
| 5    | 48,000               | 4    | 125  | 3               | 49,000       | 51,000                      | 63,500           | 25               |
| 6    | 36,000               | 4    | 150  | 0               | 37,300       | 42,300                      | 63,500           | 25               |
| 7    | 48,000               | 4    | 150  | 4               | 48,300       | 50,700                      | 63,600           | 27               |
| 8    | 36,000               | 4    | 175  | 0               | 38,100       | 44,600                      | 63,600           | 25               |
| 9    | 48,000               | 4    | 175  | 5               | 51,800       | 55,800                      | 62,000           | 22               |
| 10   | 36,000               | 4    | 200  | 0               | 50,000       | 58,300                      | 65,800           | 13               |
| 11   | 45,000               | 4    | 200  | 5               | 54,800       | 61,200                      | 65,200           | 12               |
| 12   | 36,000               | 4    | 225  | 0               | 49,400       | 57,500                      | 64,600           | 11               |
| 13   | 30,000               | 4    | 250  | 0               | 41,200       | 48,300                      | 58,600           | 10               |

TABLE 14  
Properties of aluminum alloy 24ST  
after stress-aging

| Line | Stress-Age Treatment |      |      | Creep,<br>Per Cent | Prop'l<br>Limit | 0.2% Off-<br>set Yield<br>Strength | Tensile<br>Strength | Elong.,<br>Per Cent |
|------|----------------------|------|------|--------------------|-----------------|------------------------------------|---------------------|---------------------|
|      | Stress,<br>p. s. i.  | Hrs. | ° C. |                    |                 |                                    |                     |                     |
| 1    | None                 |      |      |                    | 38,000          | 49,750                             | 69,300              | 17                  |
| 2    | 38,000               | 4    | 100  | 0                  | 40,400          | 50,300                             | 71,800              | 17                  |
| 3    | 49,500               | 4    | 100  | 0                  | 48,700          | 51,300                             | 70,000              | 20                  |
| 4    | 38,000               | 4    | 125  | 0                  | 41,000          | 49,300                             | 69,800              | 19                  |
| 5    | 49,900               | 4    | 125  | 1                  | 51,200          | 53,700                             | 69,900              | 17                  |
| 6    | 38,000               | 4    | 150  | 0                  | 44,300          | 49,900                             | 70,300              | 20                  |
| 7    | 49,500               | 4    | 150  | 0                  | 48,800          | 52,000                             | 69,800              | 18                  |
| 8    | 38,000               | 4    | 175  | 0                  | 40,300          | 49,200                             | 69,300              | 18                  |
| 9    | 49,000               | 4    | 175  | 1                  | 51,500          | 53,300                             | 69,300              | 19                  |
| 10   | 38,000               | 4    | 200  | 0                  | 45,500          | 55,000                             | 70,200              | 14                  |
| 11   | 45,000               | 4    | 200  | 1                  | 51,300          | 55,500                             | 69,400              | 13                  |
| 12   | 38,000               | 4    | 225  | 0                  | 51,000          | 62,500                             | 69,300              | 5                   |
| 13   | 30,300               | 4    | 250  | 0.5                | 43,800          | 52,200                             | 60,000              | 5                   |

Line 1, Table 14, gives the tensile properties for this alloy in its normally heat-treated condition. Lines 3 and 7 give two, practically equivalent, preferred stress-aging treatments for maximum elastic properties (without destructive creep). The proportional limit is increased by about 27%, and the yield strength by about 5%, with elongation increased slightly. If higher ductility and shock resistance are not required in a given application, the stress-aging treatment of line 12 might be preferred.

to stress age to at least double their proportional or elastic limits. Lesser savings apply to those alloys of smaller inherent stress-ageability.

What I claim as new and desire to secure by Letters Patent of the United States is:

1. The method for improving the properties of an alloy consisting wholly or in major part of one or more solid solution phases which comprises artificially aging said alloy for from 15 minutes to 20 hours at a temperature below but within 100° C. of the recrystallization tempera-

30

TABLE 15  
Properties of aluminum alloy 75ST  
after stress-aging

| Line | Stress-Age Treatment |      |      | Creep,<br>Per Cent | Prop'l<br>Limit | 0.2% Off-<br>set Yield<br>Strength | Tensile<br>Strength | Elong.,<br>Per Cent |
|------|----------------------|------|------|--------------------|-----------------|------------------------------------|---------------------|---------------------|
|      | Stress,<br>p. s. i.  | Hrs. | ° C. |                    |                 |                                    |                     |                     |
| 1    | None                 |      |      |                    | 57,700          | 71,500                             | 82,000              | 11                  |
| 2    | 58,000               | 4    | 100  | 0                  | 61,600          | 71,900                             | 83,800              | 14                  |
| 3    | 58,000               | 4    | 125  | 0                  | 60,000          | 72,200                             | 82,000              | 13                  |
| 4    | 58,000               | 4    | 150  | 0                  | 65,800          | 73,700                             | 81,000              | 11                  |
| 5    | 50,200               | 4    | 175  | 1                  | 61,000          | 70,500                             | 77,000              | 10                  |
| 6    | 35,000               | 4    | 200  | 0                  | 48,900          | 58,700                             | 68,500              | 7                   |
| 7    | 25,000               | 4    | 225  | 0.5                | 35,700          | 42,300                             | 54,000              | 5                   |

Line 1, Table 15, gives the tensile properties for this alloy in its normally heat-treated condition. Line 4 gives the preferred stress-aging treatment for maximum elastic properties. The proportional limit is increased by about 16% with no loss in elongation.

The true explanation for the remarkable results of the new stress-aging treatment has not been wholly or definitely determined. A considerable change in crystal structure seems necessarily involved but it could well be submicroscopic. It has been observed that cold worked structures stress-aged take five to ten times as long to etch and give very sharp structures for clear focussing whereas plain cold worked structures are impossible of sharp focussing at magnifications as high as 2000 diameters. Variations in structure, such as segmentation of slip bands and apparent precipitation have been observed but not proved. A lattice ordering reaction may be involved in some instances.

One advantage of my improved stress-aging process is that present operational stresses can be borne by half the present cross sections or even less if the operating parts are stress-aged and also that present operating parts can support twice the present operational stress or even more if the parts are stress-aged. This 2:1 ratio applies for the many alloys that have the capacity

ture and under an externally applied stress at least equal to the proportional limit but not exceeding the 0.2% offset yield strength of said alloy prior to said aging.

2. The method for improving the properties of an alloy consisting principally of one or more solid solution phases which comprises artificially aging said alloy at a temperature below but within 100° C. of the recrystallization temperature for at least 15 minutes under an externally applied stress between the proportional limit and 0.2% offset yield strength of said alloy prior to said aging.

3. The method for improving the properties of an alloy consisting principally of one or more solid solution phases which comprises artificially aging said alloy at a temperature below but within 100° C. of the recrystallization temperature for from 4 to 20 hours under an externally applied stress which is at least equal to the proportional limit and does not exceed the 0.2% offset yield strength of said alloy prior to said aging.

4. The method for improving the properties of an alloy consisting principally of one or more solid solution phases, which comprises aging said alloy at a temperature below but within about 100° C. of the recrystallization temperature of said alloy for from 15 minutes to 4 hours and under an externally applied stress which is at

60

70

65

75

least equal to the proportional limit of said alloy prior to said aging and which is insufficient to cause a permanent deformation of more than one mil per inch.

5. The method for improving the properties of an alloy consisting principally of one or more solid solution phases which comprises aging said alloy for one-quarter to twenty hours at a temperature within the range of from 100° C. below the recrystallization temperature up to the recrystallization temperature of said alloy and under an externally applied stress at least equal to the proportional limit of said alloy and not exceeding the 0.2% offset yield strength of the alloy prior to said aging, the time, temperature and stress conditions being such that no practically measurable permanent deformation of the alloy is effected.

6. The method for improving the properties of an alloy consisting principally of one or more solid solution phases, which comprises artificially aging said alloy under an externally applied stress within the range of the proportional limit and the 0.2% offset yield strength determined for said alloy in its condition preceding aging, said stress being applied to said alloy for at least fifteen minutes at a temperature below but within 100° C. of the recrystallization temperature.

7. The method for improving the properties of an alloy consisting principally of one or more solid solution phases, which comprises applying an external stress to said alloy while it is aged at a temperature below but within about 100° C. of the recrystallization temperature of said alloy, said stress being within the range between the proportional limit of said alloy and its 0.2% offset yield strength determined for the alloy in the condition preceding aging, and cooling said alloy to room temperature under said applied stress.

8. The method for improving the properties of a copper base alloy consisting principally of one or more solid solution phases, which comprises artificially aging said alloy at a temperature of from 175 to 275° C. under an externally applied stress within the range of the proportional limit and the 0.2% offset yield strength as determined for said alloy in its condition preceding aging, said stress being applied to said alloy for from 15 minutes to 4 hours.

9. The method for improving the properties of a copper base alloy wire consisting principally of one or more solid solution phases, which comprises applying an external stress to said wire for from 15 minutes to 4 hours while it is aged at a temperature below but within about 100° C. of the recrystallization temperature of said alloy, said stress being within the range between the proportional limit of said alloy and its 0.2% offset yield strength as determined for the alloy in the condition preceding aging, the time, stress and temperature conditions being insufficient to effect

any practically measurable permanent deformation of said alloy.

10. The method of claim 8 wherein the copper base alloy is a cold worked brass.

11. The method for improving the properties of a ferrous alloy which consists principally of one or more solid solution phases, which comprises artificially aging said alloy at a temperature below but within 100° C. of the recrystallization temperature under an externally applied stress within the range of the proportional limit and the 0.2% offset yield strength as determined for said alloy in its condition preceding aging, said stress being applied to said alloy for from 15 minutes to 4 hours.

12. The method for improving the properties of a stainless steel, which comprises applying an external stress of about 90,000 p. s. i. to said alloy for from 15 minutes to 20 hours while it is aged at a temperature of about 400° C. and cooling said alloy to room temperature under said applied stress.

13. The method of claim 12 wherein the stress is applied for from 15 minutes to 4 hours.

14. The method for improving the properties of an aluminum base alloy consisting principally of one or more solid solution phases, which comprises artificially aging said alloy at a temperature of from 100 to 200° C. under an externally applied stress within the range of the proportional limit and the 0.2% offset yield strength as determined for said alloy in its condition preceding aging, said stress being applied to said alloy for from 15 minutes to 4 hours.

15. The method for improving the properties of a cold worked aluminum base alloy consisting principally of one or more solid solution phases, which comprises applying an external stress to said alloy for from 15 minutes to 20 hours while it is aged at a temperature below but within the range of from 100° C. below the recrystallization temperature up to the recrystallization temperature of said alloy, said stress being within the range between the proportional limit of said alloy and its 0.2% offset yield strength as determined for the alloy in the condition preceding aging, and cooling said alloy to room temperature under said applied stress.

RICHARDS H. HARRINGTON.

#### REFERENCES CITED

The following references are of record in the file of this patent:

#### UNITED STATES PATENTS

| Number    | Name           | Date          |
|-----------|----------------|---------------|
| 1,887,339 | Stroble _____  | Nov. 8, 1932  |
| 1,942,025 | Frost _____    | Jan. 2, 1934  |
| 2,261,878 | Hathaway _____ | Nov. 4, 1941  |
| 2,351,922 | Burgwin _____  | June 20, 1944 |